

G. S. DEY.  
LENS FORMING PROCESS.  
APPLICATION FILED JAN. 3, 1920.

1,416,947.

Patented May 23, 1922.



INVENTOR  
GILBERT S. DEY

BY

H. H. Styll & H. Parsons  
ATTORNEYS

# UNITED STATES PATENT OFFICE.

GILBERT S. DEY, OF SOUTHBIDGE, MASSACHUSETTS, ASSIGNOR TO AMERICAN OPTICAL COMPANY, OF SOUTHBIDGE, MASSACHUSETTS, A CORPORATION OF MASSACHUSETTS.

## LENS-FORMING PROCESS.

1,416,947.

Specification of Letters Patent. Patented May 23, 1922.

Application filed January 3, 1920. Serial No. 349,292.

To all whom it may concern:

Be it known that I, GILBERT S. DEY, a citizen of the United States, residing at Southbridge, in the county of Worcester and State 5 of Massachusetts, have invented certain new and useful Improvements in Lens-Forming Processes, of which the following is a specification.

This invention relates to new and improved processes of forming ophthalmic lenses and has particular reference to lenses of the toric type as being the more difficult to construct at the present time, although it will be understood that it is equally applicable to spherical, bifocal and other forms 10 of lens blanks.

One of the leading objects of the present invention is the provision of a novel and improved process through the use of which 20 the lens may be satisfactorily dropped to the correct shape without the injurious effects on the surface caused by moulding of the lens in this form, and consequently a process which will serve to reduce the grinding of the toric or other difficult to produce surfaces to a minimum.

Another object of the invention is the provision of a novel and improved process for forming blanks of this character in which 30 the axis of the cylinder, in the case of a cylinder or toric blank, will be clearly, exactly and indelibly marked or denoted so that the lens may be subsequently readily finished and the intended cylinder axis maintained, 35 thus both increasing the speed of production and lessening the cost of production of the lens of the type in question.

Other objects and advantages of my construction should be readily apparent by reference to the following specification taken 40 in connection with the accompanying drawings, and it will be understood that I may make any modifications in the specific details of construction shown and described within 45 the scope of the appended claims without departing from or exceeding the spirit of my invention.

Figure I represents a plan view of one of the mould members or supports, showing 50 certain glass pieces in position thereon.

Figure II represents a transverse sectional view as on the line II-II of Figure I, showing a lens in its initial position.

Figure III represents a longitudinal sec- 55 tional view on the line III-III.

Figure IV represents a sectional view of the lens at one step in my process.

Figure V represents a plan view thereof at a further step in the process.

Figure VI represents a sectional view of 60 the construction shown in Figure V.

Figure VII represents a sectional view of a subsequent step in the process.

Figure VIII represents a sectional view of 65 a different form of mould member.

Prior to my present invention the most common way of producing what is known as toric or like lenses having two powers in the opposite meridian has been by the grinding of ordinary glass blanks which have been 70 pressed in moulds to secure a certain general curvature, the toric surface being ordinarily roughed out in some suitable manner to produce a closer approximation to the toric curve, and then being given suitable relative 75 motion over a tool bearing the curves which it is desired to transfer contragenerically to the glass.

The purpose of my invention, however, is to do away to the largest possible degree 80 with this preliminary work and to reduce to a minimum the necessary grinding on the toric face of the lens, in that certain difficulties are inherent in grinding toric surfaces not met with in plain surfaces.

In the accomplishment of this result I first preferably polish on both sides the glass blank 1, after which I mount it upon a suitable former 2, which may be a carborundum or other slab suitably surfaced and provided with the 85 necessary curve or curves according to the particular curves which the final lens is desired to have.

Inasmuch as the toric surface is the one which is primarily considered, and as my process is particularly applicable in 90 the factory production of what is known as toric blanks, that is, blanks with the toric side finished, the spherical side remaining to be ground, I prefer to make use of such form of mould or former 2, as will not come 95 into contact with what is to be the final toric surface but only come in contact with the opposite surface of the glass blank.

Ordinarily the toric curve is placed on the inner face of the glass and in these cases I find it 100 particularly advantageous to make use of concave mould or former faces 3 on the member 2, which in this case are not of the curve or curves to be produced on the toric face of the glass, but are so calculated that 105

Figure I represents a plan view of one of the mould members or supports, showing 50 certain glass pieces in position thereon.

if a flat piece of glass be placed on the former and caused by heat to drop down to fit the former, the curves resultant from the shape of the mould and the thickness of the glass 5 together produced upon the upper or non-contacting face of the blank will be substantially the curves desired.

The production of the exact curves can, of course, be accomplished by dropping the 10 blank over a convex form member 4, such as is illustrated in connection with Figure VIII, the disadvantage of this form, however, being that it is necessary to employ the side members 5 with the adjusting screw 15 6 carefully set to maintain the blank in exact correct position against any lateral slipping movement, while in the case of Figures I and II of the drawings the side members 5 and adjusting devices 6 are shown and may 20 be employed for ordinary conditions but this is not entirely necessary since the concave former will of itself serve to steady and prevent undue lateral or longitudinal sliding movement on the glass. In any 25 event, the glass blank, as before stated, preferably of polished condition, being placed on the former, the former and blank are subjected to heat to soften the glass so the glass will drop down to and at its contacting 30 surface assume the shape of the former, although as before mentioned the former may be so calculated as with the glass thickness added to produce any desired curve or curves on the upper face of the glass if that 35 is the face which is to be subsequently first finished.

It will be understood that it is of extreme importance that the cylinder axis be maintained during the subsequent grinding or 40 polishing operations as if the tool and lens are not placed for these operations in exact correct relationship then the advantage gained by the first steps in my process will be lost and initial amounts of glass will have 45 to be removed. To, therefore, insure correct subsequent operations I preferably place on one face of the glass 1, the axis designations 7 coinciding with the axis of the former 2, and if desired the numerals 8 50 designating the dioptric values of the curves which are to be produced on this face of the glass my moulding. For this purpose I use a fusible enamel which may be quickly and easily applied before heating the glass, and 55 which as the glass is heated will maintain its regular form but will be fused into the glass and become united therewith as an integral part thereof, thus continuing to designate the axis of the glass until the fusible 60 enamel has been entirely ground away or removed. After the dropping and line fusing operation has been completed the glass is then taken to a grinding tool where the toric surface 9 may be ground and polished, or merely polished, as the necessity 65

may be, when the blank may be sold in this form with the surface 10 still in roughened condition from contact with the mould if desired, or the surface 10, if this be the toric one, which has been in contact with the mould, may be ground and polished when the semi-finished blank, as it is termed in the trade, will be found to be substantially transparent and capable of ready examination for the determination of interior defects before the final curve is placed on the opposite side thereof.

I claim:

1. As an article of manufacture, a dropped toric ophthalmic lens blank having axis designations fused thereon by the heat of the dropping operation.

2. The process of forming a toric lens consisting in shaping a form with a toric surface, placing the glass material on the form, placing fusible axis designations on the glass, and subjecting the parts to heat to cause the glass to assume toric form and the fusible designations to unite with the glass and permanently indicate the cylinder axis which has been produced on the glass by the dropping process.

3. The process of forming a toric lens blank consisting in constructing a form, calculating the curves on the form to allow for predetermined glass thickness, grinding the glass to the predetermined thickness while in plano form, placing the glass thus ground on the toric form, and dropping the glass to produce on the free surface the calculated curve.

4. The process of forming a toric lens blank consisting in constructing a form, calculating the curves on the form to allow for predetermined glass thickness, grinding the glass to the predetermined thickness while in plano form, placing the glass thus ground on the toric form, marking suitable designations on the exposed face of the glass, and dropping the glass on the form to produce the predetermined surface.

5. The process of forming a toric lens blank consisting in constructing a form; calculating the curves on the form to allow for predetermined glass thickness, grinding the glass to the predetermined thickness while in plano form, placing the glass thus ground on the toric form, marking suitable designations on the exposed face of the glass, dropping the glass on the form to produce the predetermined surface, and subsequently grinding and polishing the surface injured by the dropping process.

6. The process of dropping glass blanks, consisting in preparing a form with a plurality of glass receiving recesses, polishing glass in plano form, placing the plano glass in sections above the several recesses, placing suitable designations of fusible material on the blanks, and subjecting the parts

to heat to cause the glass to drop down to and assume the curve of the form and the designations to permanently unite with the glass, and subsequently grinding the glass on the form engaging side to restore its curve and finishing the glass on the opposite surface in accordance with the designations appearing thereon.

7. The process of dropping glass blanks, 10 consisting in preparing a form with a plurality of glass receiving recesses, polishing glass in plano form, placing the plano glass in sections above the several recesses, placing suitable designations of fusible material 15 on the blanks, and subjecting the parts to heat to cause the glass to drop down to and assume the curve of the form and the designations to permanently unite with the glass, subsequently grinding the glass on the 20 form engaging side to restore its curve, finishing the glass on the opposite surface in accordance with the designations appearing thereon, and continuing this finishing operation until the designations are obliterated 25 from the field of vision of the lens.

8. The process of forming ophthalmic lenses, including shaping a form with predetermined curves, providing side members for the form to prevent lateral slipping of 30 the glass, mounting the glass upon the form

between the side members, and subjecting the parts to heat to cause the glass to settle down onto the form between the side members and assume the shape of the form.

9. The process of forming ophthalmic 35 lens blanks, including producing predetermined configurations on a form, providing lateral guides and adjustment members for the form, positioning a glass blank over the form through the use of the lateral and adjusting members, and dropping the lens to the curve of the mould under the influence of heat when properly positioned to produce a predetermined blank.

10. As an article of manufacture a dropped 45 cylinder lens blank having axis designations thereon of a fusible cement, said axis designations being permanently united with the glass by the action of the heat required for dropping the blank to cylinder form.

11. As an article of manufacture a cylinder lens blank having axis designations fused on the cylinder face thereof.

In testimony whereof I have affixed my signature, in presence of two witnesses.

GILBERT S. DEY.

Witnesses:

H. K. PARSONS,  
ALICE G. HASKELL.